

Patented Jan. 5, 1926.

## Cross Reference

Examiner

1,568,234

## UNITED STATES PATENT OFFICE.

DANIEL H. MELOCHE, OF DETROIT, MICHIGAN, ASSIGNOR TO EARL HOLLEY, OF DETROIT, MICHIGAN.

## COATING FOR MOLDS.

No Drawing.

Application filed January 12, 1924. Serial No. 685,898.

22-189

To all whom it may concern:

Be it known that I, DANIEL H. MELOCHE, a citizen of the United States, residing at 3248 Fourth Avenue, Detroit, in the county of Wayne and State of Michigan, have invented certain new and useful Improvements in Coatings for Molds, of which the following is a specification.

This invention relates to an improved coating for the protection of the surface of metal molds exposed to molten metal. The specific object of this invention is to provide means whereby the sprues and other portions of the metal molds used in the production of non-ferrous castings may be protected from the erosive action of said non-ferrous metals. Another object is to maintain the metal in the sprues molten so as to prevent "piping" in the casting.

The difficulty heretofore found when casting non-ferrous metals in molds, which are usually made of iron or steel, is that the non-ferrous metals attack the iron or steel molds and eventually destroy them, especially in the sprue and gates, there being quite a considerable chemical affinity between the iron molds and the metals cast therein. I have discovered that the coating, to be described hereafter, acts as an effective barrier against the molten metals and thus protects the iron molds so that the life of the iron molds is extended indefinitely. Another difficulty is that piping or porosity results from the premature freezing of the sprue.

I have discovered that if finely ground fire clay be suspended in water in which a little water-glass is dissolved, and to this suspension a little lampblack be added, that this mixture of dilute water-glass, fire clay, and lampblack constitutes a very satisfactory wash, and a cheap cast iron mold so coated is superior to an expensive uncoated steel mold. In order to make this wash adhere to the molds it is only necessary that the molds be higher than 250° F., and that the temperature of the mold be maintained

above that temperature during the coating period. This merely means that heat must be applied between each coat.

By having the wash relatively thin a great number of coats are required, and the greater the number of coats the more adherent and therefore the more resistant is the coating to the erosive action of the non-ferrous metals cast in the molds.

Satisfactory results have been obtained by using a 10% saturated solution of sodium silicate in water and mixing with this solution an equal weight of finely ground fire clay and lampblack. The proportion of fire clay and lampblack should be two parts of fire clay to one part of lampblack. This mixture, consisting of approximately 45% water, 5% sodium silicate, 33% fire clay, and 17% lampblack, is the thickest wash that I use.

By increasing the quantity of water, without increasing the proportions of the other elements, I obtain a thinner wash which is more satisfactory when relatively intricate molds have to be protected. For simple molds, such as a piston mold, and for protecting the sprue the percentages given above are satisfactory.

One advantage of protecting the sprue with this heat-insulating coating is that the metal in the sprue stays molten longer and thus feeds the casting, so as to fill up any cavities which would otherwise form due to contraction.

What I claim is:

1. A coating for protecting iron molds, consisting of an inert refractory insulating material mixed with lampblack and a small percentage of soluble silicate acting as a binder only, for the lampblack and the refractory insulating coating.

2. A coating for semipermanent molds to be used for the production of non-ferrous castings, consisting of fire clay, lampblack, and a heat-resisting adhesive.

3. An insulating refractory wash for coating semipermanent molds, consisting

of lampblack and fire clay suspended in water in which there is dissolved a small percentage of heat-resisting binder.

4. A metal mold for the production of 5 non-ferrous castings, said mold being lined with a smooth adherent coating of fire clay, lampblack, and an inorganic heat-resisting binder.

5. A metal mold for the production of non-ferrous castings, said mold being lined 10 with a smooth adherent coating of fire clay and lampblack, together with a binder of soluble silicate.

In testimony whereof I affix my signature.

DANIEL H. MELOCHE.